

# United States Patent Office

2,860,953

Patented Nov. 18, 1958

1

2,860,953

## CORROSION INHIBITION OF TITANIUM-BASE MATERIALS BY FUMING NITRIC ACID

Howard B. Bomberger, East Liverpool, Ohio, assignor, by mesne assignments, to Crucible Steel Company of America, Flemington, N. J., a corporation of New Jersey

No Drawing. Application July 19, 1956  
Serial No. 598,743

7 Claims. (Cl. 23—157)

This invention relates to fuming nitric acid compositions with decreased ability to cause corrosion and stress corrosion cracking of titanium and titanium base materials. In another aspect, it relates to methods of inhibiting corrosion and stress corrosion cracking of titanium base materials by red fuming nitric acid.

Titanium is well known for its unusually high resistance to corrosion by most chemicals. Likewise, the titanium base materials, i. e., titanium alloys containing a major portion of titanium, are also quite resistant to corrosion. The term titanium base material as employed herein is intended to include not only titanium alloys but also the unalloyed metal. These materials originally appeared ideally suited as containers for nitric acid solutions of all concentrations, and considerable interest developed in the use of titanium base components in the handling of nitric acid of very high concentration, more particularly, red fuming nitric acid. Early studies indicated that these materials possessed excellent corrosion resisting properties in the presence of this acid. However, later more exhaustive investigations detected instances where the corrosion rate was abnormally high. That is to say, the usual low rate of less than 0.1 mil penetration per year, which is considered acceptable, was exceeded many times. These tests also established that the titanium alloys tend to corrode at a much higher rate in the presence of red fuming nitric acid than unalloyed titanium.

Early corrosion studies of titanium and its alloys in the presence of red fuming nitric acid indicated that corrosion is accomplished by formation on the metal surface of an adherent, dark, generally black, corrosion product which is pyrophoric. This substance can be detonated in an oxidizing environment by shock, heating, or by an electric spark. When removed from the surface of the metal, it can be similarly detonated. Its sensitivity to impact is approximately equal to that of nitroglycerine and mercury fulminate. The black corrosion product has been identified as very finely divided titanium metal, and is the result of extensive intergranular corrosion. Its sensitivity has resulted in at least one fatal accident, and has caused considerable reluctance to employ light weight titanium and titanium alloys as containers for red fuming nitric acid.

In addition to formation of the pyrophoric surface coating, the metal has been found to undergo considerable stress corrosion cracking in the presence of the fuming acid. This cracking is particularly evident around number stamps and other identifying marks and notches, as well as at the sheared edges of test samples. The titanium alloys are considerably more susceptible to stress corrosion cracking than is commercially pure titanium metal.

While considerable work has been done identifying the corrosion product, investigating the susceptibility of titanium base materials to corrosion cracking, measuring corrosion rate and correlating corrosion and cracking rates with the  $\text{NO}_2$  and water concentration of the fuming

2

nitric acid, as yet there has been nothing published regarding methods or compositions for inhibiting or substantially eliminating the corrosion. Accordingly, methods of inhibiting titanium base corrosion, and/or a modified fuming nitric acid solution which would not corrode titanium and its alloys would be highly desirable.

The present invention provides two methods for substantially eliminating serious corrosion and stress corrosion cracking of titanium base materials by fuming nitric acid in sealed containers, as well as a modified red fuming nitric acid composition of substantially reduced ability to corrode these materials.

The first of these methods, referred to as the oxygen method, comprises providing a vapor space above the red fuming nitric acid in the sealed titanium base vessel and maintaining the concentration of oxygen in this vapor zone at least equal to 5% by volume. In the case of titanium base acid containers open to the atmosphere, no precautions need be taken, since there is sufficient oxygen in the air to provide the required oxygen concentration at the liquid-vapor interface. The titanium base acid containers find their widest application where sealed. In closed containers, as will be shown in the tables hereinafter, corrosion of the metal is rapid with substantial formation of the pyrophoric corrosion product and extensive corrosion cracking.

I have found that corrosion can be substantially arrested and cracking prevented by periodically flushing the vapor zone provided in the container with air or commercial oxygen in order to maintain the oxygen concentration in this vapor zone at least 5% by volume. The presence of oxygen at the liquid-vapor interface is a most effective inhibitor. While air may be satisfactorily employed, I prefer commercial oxygen for best results. Although a minimum of 5% oxygen by volume at the liquid-vapor interface is sufficient to arrest and satisfactorily control corrosion, the oxygen concentration may vary widely above this figure even to as much as 100% oxygen in the vapor zone. It is preferable to flush the vapor zone periodically with oxygen in high concentration, since flushing may then be at relatively widely spaced intervals as distinguished from the frequency necessary when air containing only about 20% oxygen is employed. Of course, the required frequency of flushing, whether with oxygen or air, will depend upon the relative volumes of the vapor zone and acid, and the area of the liquid-vapor interface. In tests which I have conducted, the volume of the vapor zone was about 25% of the total container volume, and flushing was effected daily with a volume of oxygen at atmospheric pressure about equal to the total container volume. However, these tests were not carried out in order to formulate a flushing frequency in hours or days, and it should be remembered that the controlling factor is the minimum oxygen concentration at the interface, which should not be allowed to fall below 5%.

While the mechanism by which oxygen prevents corrosion is not yet fully apparent, and I do not wish to be limited or otherwise prejudiced by an explanation, there is reason to believe that small amounts of  $\text{NO}_2$  and  $\text{HNO}_3$  are reduced to  $\text{NO}$  and  $\text{HNO}_2$  in the metal container. These latter materials appear to accelerate corrosion, and apparently in the presence of oxygen at the liquid-vapor interface, they are reoxidized before their effect on corrosion becomes appreciable.

While the above-described oxygen method quite adequately arrests, and in effect eliminates corrosion and formation of the undesirable pyrophoric product and stress corrosion cracking in titanium base materials, a periodic flushing with air or oxygen to maintain the required oxygen concentration at the interface is a bur-

densive technique, and means for flushing the containers may not always be available. The other method by which I am able to substantially eliminate corrosion overcomes the necessity for periodically changing the atmosphere in the container, and also eliminates the necessity for the vapor zone thus permitting complete filling of the container. By this second method, an inhibitor is added and dissolved or is otherwise present in the fuming nitric acid.

I have found that certain metal ions, in their highest degree of oxidation when present in very small concentration in the fuming nitric acid, substantially reduce corrosion and cracking of titanium base materials. More particularly, I have found that the presence of cupric, chromic, ferric, manganic and stannic ions as well as mixtures of one or more of these ions in the fuming nitric acid effectively inhibits corrosion. The degree of corrosion and cracking inhibition realized is entirely satisfactory, and when cupric ions are employed, inhibition is substantially the same as that afforded by the oxygen flushing method. In accordance with the present invention, these ions are added to red fuming nitric acid in the form of salts in amounts sufficient to provide a metal salt concentration at least equal to about 0.01% by weight of the acid. In some instances, a smaller amount is effective. For example, 0.008% by weight copper sulfate is adequate. This latter figure corresponds to a cupric ion concentration in the acid of about 0.003% by weight. However, for good control and long-time applications, an excess over the above 0.01% minimum can be employed without harm, and is desirable in order to prevent depletion of the inhibitor. Amounts in excess of about 2% by weight of the salt are unnecessary, and this figure appears to be a practical maximum for longtime storage conditions. About 0.1% salt is recommended for most conditions.

The metal ions employed are in their highest degree of oxidation. This is important since the metal ions in a lower state of oxidation are unstable in and are oxidized by the acid, which results in simultaneous reduction of some of the  $\text{NO}_2$  and  $\text{HNO}_3$  to  $\text{NO}$  and  $\text{HNO}_2$ , respectively. It is my belief that this reduction should be avoided since the reduction products,  $\text{NO}$  and  $\text{HNO}_2$ , appear to accelerate corrosion. For this reason, I do not introduce the metals as such or salts thereof in which the metal is not in its highest degree of oxidation.

Cupric, chromic, ferric, manganic and stannic salts, such as their oxides, bromides, iodides, carbonates, sulfates, nitrates and phosphates may be employed with

sufficiently low so as to have no effect upon corrosion rates. To a lesser extent, chloride ions also appear to interfere with the desired result, and particularly in combination with copper. On the other hand, ferric chloride is a satisfactory inhibitor. Thus, it can be said that when cupric ions are employed as the inhibitor, the acid should be substantially free of chloride ions. In addition to the binary salts indicated, complex salts, which are generally less stable, e. g., dichromates and permanganates, may be used successfully.

Several series of tests were conducted in order to establish the corrosion rate and extent of stress corrosion cracking in titanium base materials by red fuming nitric acid. The tests illustrate the effect of the metal ion inhibitors, and also the effectiveness of air and oxygen at the liquid-vapor interface.

#### EXAMPLE 1

In the first of these tests, samples of titanium metal and a titanium-7% manganese alloy both in the "as-received" and 20% cold rolled condition were immersed in 400 ml. of red fuming nitric acid (80%  $\text{HNO}_3$ , 20%  $\text{NO}_2$ ) in 570 ml. polyethylene bottles. The metal samples measured 0.050" x 0.5" x 4". One of the containers was left open to the atmosphere, while the remaining four were sealed by means of a softened paraffin block which was held in place by a five pound weight. Each of the bottles contained a titanium metal sample in the as-received and in the 20% cold rolled condition as well as two similar samples of the titanium-manganese alloy. Samples remained in the acid for 28 days at room temperature. No inhibitor was added to the acid in container 1. Container 2 contained in addition to the red fuming nitric acid 1.5% by weight of water in order to illustrate its effect upon corrosion rate. Container 3 was open to the atmosphere. Container 4 was sealed and the vapor space above the fuming nitric acid, amounting to about  $\frac{1}{4}$  the volume of the container, was flushed daily with approximately 570 ml. of oxygen at atmospheric pressure. The oxygen line to this container was destroyed by acid vapors after three weeks, so oxygen flushing was accomplished for only  $\frac{3}{4}$  of the test period. To container 5 there was added 5 grams of anhydrous copper sulfate equivalent to 0.32% by weight cupric ions.

The following table reflects the corrosion rates of the metal samples in mils per year after 28 days, the appearance of the samples following the test, and a notation regarding the stress corrosion cracking, if any, produced by the test.

Table I

| Container No. | Conditions (28 day test)                           | Corrosion Rates In Mils per Year |           |           |           | Remarks                                           |  |
|---------------|----------------------------------------------------|----------------------------------|-----------|-----------|-----------|---------------------------------------------------|--|
|               |                                                    | Titanium                         |           | Ti-7% Mn  |           |                                                   |  |
|               |                                                    | As Rec'd.                        | 20% O. R. | As Rec'd. | 20% O. R. |                                                   |  |
| 1             | Sealed                                             | 1.82                             | 1.80      | 3.04      | 3.00      | Heavy staining and cracking.                      |  |
| 2             | Sealed, 1.5% $\text{H}_2\text{O}$                  | 7.43                             | 7.15      | 11.23     | 10.72     | Heavy staining, etching and cracking.             |  |
| 3             | Open                                               | .018                             | 0.00      | 0.00      | .014      | No staining or evidence of corrosion or cracking. |  |
| 4             | Sealed + $\text{O}_2$ flushing                     | .056                             | .028      | .023      | .202      | Very slight staining. No cracking.                |  |
| 5             | Sealed + 0.32% $\text{Cu}^{++}$ as $\text{CuSO}_4$ | .009                             | .005      | 0.000     | .014      | No staining or cracking. No evidence of attack.   |  |

red fuming nitric acid, since it appears that the metal ion and not the anion of the salt is the effective inhibiting agent. However, I have found that fluorides of these metals, and fluoride ions in general, seem to interfere with inhibition. Accordingly, the fuming nitric acid is maintained substantially free of fluoride ions, that is, fluoride ions are absent or their concentration is suffi-

70 Container 1 which was sealed is taken as the standard for comparison, and it will be observed that an addition of only 1.5% by weight of water to the red fuming nitric acid increases the rate of corrosion of both the titanium and the titanium alloy from three to four times. The samples in container 3, which was open to the atmosphere and in which the oxygen concentration at the

liquid-vapor interface was substantially that of the air, corroded at a rate roughly 100 times less in the case of titanium and approximately 300 times less in the case of the alloy than the samples in sealed container 1. The samples in sealed container 4 to which oxygen was introduced daily for three of the four weeks of the test, corroded at a rate somewhat greater than those in container 3, but this can be accounted for in part by the breakdown which occurred. Nevertheless, the low rate of corrosion observed is satisfactory, and the results clearly indicate that oxygen was the element instrumental in inhibiting attack of the samples. Examination of the corrosion rate and remarks in connection with container 2, which contained the small amount of water, clearly indicates that moisture is in no way beneficial as an inhibitor and that it is oxygen and not moisture contained in the air which inhibited attack in container 3.

The 0.32% cupric ion concentration in container 5 effectively inhibited both corrosion and stress corrosion cracking, and was as effective as an open container. While the mechanism of inhibition in this case is not clearly understood, it is apparently different from the action of oxygen. Quite possibly, corrosion is prevented by adsorption of cupric ions on the surface of the titanium base material.

#### EXAMPLE 2

The second series of tests was similar to those of Example 1, but carried out over a period of only seven days. The inhibiting effect of manganese, ferric, and chro-

mic ions was observed. Each bottle contained samples of both titanium and titanium-7% manganese in the as-received condition and titanium in 20% cold rolled condition. The corrosion rates and extent of cracking are noted in Table II.

inhibiting effect of oxygen of the air. Sealed containers 3, 4 and 5 contained 5 grams of manganese dioxide, ferric chloride and chromic oxide, respectively. While it is apparent that manganic and ferric ions are not as effective as the chromic ion, each of these three ions effectively reduced corrosion rates, particularly on the titanium metal samples. The rate of reduction is somewhat less on the alloy samples. Of the three, in the ionic concentration employed, chromic ions are clearly the most effective on titanium metal and ferric ions are best for the titanium-manganese alloy.

#### EXAMPLE 3

The third series of tests was conducted in order to observe the effect of the degree of oxidation of the copper ions upon ability to inhibit corrosion. The tests were in general carried out as described in Example 1. However, the samples were of somewhat different size, namely, 0.035" x 0.3" x 4", and the duration of the test was 31 days. Each of the bottles contained 400 ml. of solution and an air vapor zone of 150 ml. All of the containers were tightly sealed by placing a 1/2" cap of paraffin over the top and weighing it with approximately 2 pounds. The results of these tests appear in Table III. The small corrosion rates recorded could in isolated instances be due to weighing errors, since a corrosion rate of 0.005 mil per year is equivalent to a weight loss of only 0.1 milligram. Consequently, where there was little weight loss, surface appearances, such as staining and cracking, are a more accurate indication of corrosion.

Table III

| Container No. | Conditions (Containers Sealed 31 day test)          | Corrosion Rate in Mils per Year |           |           |           | Remarks                                                |  |
|---------------|-----------------------------------------------------|---------------------------------|-----------|-----------|-----------|--------------------------------------------------------|--|
|               |                                                     | Ti Metal                        |           | Ti-7% Mn  |           |                                                        |  |
|               |                                                     | As Rec'd.                       | 20% C. R. | As Rec'd. | 20% C. R. |                                                        |  |
| 1             | RFNA only                                           | .092                            | .054      | .007      | .070      | Heavy staining and corrosion.                          |  |
| 2             | RFNA + 0.003% Cu <sup>++</sup> as CuSO <sub>4</sub> | .005                            | .016      | .054      | .087      | No staining.                                           |  |
| 3             | RFNA + 0.06% Cu <sup>++</sup> as CuSO <sub>4</sub>  | .032                            | .022      | -----     | .24       | Do.                                                    |  |
| 4             | RFNA + .06% Cu <sup>+</sup> as CuCl <sub>2</sub>    | .033                            | .038      | -----     | .37       | No staining. Cracking on all but as-received titanium. |  |
| 5             | RFNA + 0.06% Cu metal                               | .016                            | .022      | .31       | .79       | Do.                                                    |  |

mic ions was observed. Each bottle contained samples of both titanium and titanium-7% manganese in the as-received condition and titanium in 20% cold rolled condition. The corrosion rates and extent of cracking are noted in Table II.

No visible surface changes occurred in the titanium metal or the alloy in containers 2 and 3 which contained cupric ions. The presence of copper in the form of cuprous chloride in container 4 in amount equivalent to the cupric ion concentration of container 3 prevented stain-

Table II

| Container No. | Conditions (7 day test)                                     | Corrosion Rates in Mils per Year |           |           |           | Remarks                                                                                                               |  |
|---------------|-------------------------------------------------------------|----------------------------------|-----------|-----------|-----------|-----------------------------------------------------------------------------------------------------------------------|--|
|               |                                                             | Titanium                         |           | Ti-7% Mn  |           |                                                                                                                       |  |
|               |                                                             | As Rec'd.                        | 20% C. R. | As Rec'd. | 20% C. R. |                                                                                                                       |  |
| 1             | Sealed                                                      | 3.00                             | 1.21      | 11.25     | -----     | Heavy staining with corrosion product covering the surface. Extensive cracks developed at stampings and rolled edges. |  |
| 2             | Open                                                        | 0.070                            | 0.090     | 0.090     | -----     | No tarnishing or corrosion. Two minute cracks developed on the C. R. Ti sample several weeks after tests.             |  |
| 3             | Sealed + 5 gms. MnO <sub>2</sub> (0.5% Mn <sup>4+</sup> )   | 0.95                             | 0.10      | 7.5       | -----     | Slight staining. Cracks developed at stampings and rolled edges.                                                      |  |
| 4             | Sealed + 5 gms. FeCl <sub>3</sub> (0.27% Fe <sup>3+</sup> ) | 0.75                             | 1.25      | 2.85      | -----     | Slight staining. Cracks developed at rolled edges only.                                                               |  |
| 5             | Sealed + 5 gms. CrO <sub>3</sub> (0.4% Cr <sup>6+</sup> )   | 0.07                             | 0.107     | 6.32      | -----     | Very slight staining. Cracks developed at stampings and rolled edges.                                                 |  |

Container 1 illustrates uninhibited corrosion rates, while container 2, which was open, again illustrates the

ing on all of the samples, but stress corrosion cracking occurred in all samples except the as-received titanium

metal. Since dilute hydrochloric acid has been found to cause rapid stress corrosion cracking under certain conditions, it is believed that cracking of the samples in container 4 was caused for the most part by the chloride ion. The presence of cupric ions following oxidation definitely had an effect on controlling staining. Examination of the samples from container 5 containing metallic copper revealed no staining, but all except the as-received titanium metal developed cracks. Since metallic copper reduces nitric acid, reduction products of red fuming nitric acid such as NO and  $\text{HNO}_2$  are formed. These reduction products are regarded as undesirable in controlling corrosion, and it is believed that metallic copper in this manner defeats the purpose of the present invention.

The present invention thus provides needed methods for inhibiting corrosion of titanium base materials by fuming nitric acid, and these materials need no longer be considered unsafe in the handling and storage of this acid. Of the metallic ions specified herein which may be effectively employed, cupric ions are generally preferred.

What is claimed is:

1. A method of inhibiting the corrosion of titanium base material by red fuming nitric acid, which comprises incorporating with said fuming nitric acid at least about 0.01% by weight of a salt of a metal in its highest degree of oxidation selected from the group consisting of copper, chromium, iron, manganese, tin and mixtures thereof, and maintaining said acid substantially free of fluoride ions.
2. A method of inhibiting the corrosion of titanium and titanium-containing alloys by red fuming nitric acid, which comprises incorporating with said acid a cupric salt in amount sufficient to provide a concentration therein of at least about 0.003% by weight cupric ions, and maintaining said acid substantially free of fluoride ions.

3. A method of inhibiting corrosion and stress corrosion cracking of titanium base material by red fuming nitric acid, which comprises incorporating with said acid a cupric salt having an anion selected from the group consisting of sulfate, nitrate, oxide, phosphate, iodide and bromide in amount sufficient to provide a cupric ion concentration in said acid of at least about 0.003% by weight, and maintaining said acid substantially free of fluoride ions.

4. The method as set forth in claim 3, wherein the cupric salt is cupric nitrate, and the weight of salt added is at least about 0.01% by weight of the fuming nitric acid.

5. A method of inhibiting corrosion and stress corrosion cracking of titanium base material by red fuming nitric acid, which comprises incorporating with said acid cupric sulfate in amounts sufficient to provide a cupric ion concentration in said acid of at least about 0.003% by weight, and maintaining said acid substantially free of fluoride ions.

6. The method as set forth in claim 1 wherein the metal salt is added in amounts between about 0.01 and 2% by weight of the red fuming nitric acid.

7. A method of inhibiting the corrosion of titanium and titanium base alloys by red fuming nitric acid, which comprises incorporating with said acid at least about 0.01% by weight ferric chloride, and maintaining said acid substantially free of fluoride ions.

30 References Cited in the file of this patent

"The Electrochemical Society," Preprint 81-16 (1942), page 224.

"Journal of the Electrochemical Society," vol. 99, No. 1, January 1952, pages 13-15.

35 Specification Catalog of July 1951, J. T. Baker Chemical Co., Phillipsburg, New Jersey, page 146.